

Patented July 15, 1930

1,770,697

# UNITED STATES PATENT OFFICE

SHINJIRO HORII, OF TOKYO, JAPAN

## STENCIL SHEET

No Drawing.

Application filed October 8, 1927. Serial No. 225,028.

My invention relates to improvements in stencil sheets for use in duplicating manuscript and typewritten documents, drawings and like, consisting of a sheet of fibrous material coated or impregnated with a coating composition which is impermeable to ink and can be stencilized by the pressure of the stylus or the impact of the type of a writing machine.

10 It has previously been proposed to provide a stencil sheet of this kind, such as a base of fibrous material coated with a medium which includes a cellulose ester, such as cellulose nitrate or acetate, and a tempering agent, such as castor oil or other oily materials.

15 It has furthermore been proposed to provide such a stencil sheet of a fibrous base, such as yoshino paper, which is coated with a composition including a derivative of cellulose, 20 oxy cellulose or hydro-cellulose, the substance or composition being dissolved in a volatile solvent, such as ether-alcohol mixture, amyl acetate, and a tempering agent, such as resins, fatty oils, solid fatty acids and similar hydrocarbons.

25 It has furthermore been proposed to provide a stencil sheet adapted to be impressed by type and comprising a porous base having a coating which includes a gelatinizing organic colloid, such as gelatine, dispersable in water, in association with an oily material such as sperm oil as the main tempering agent, and a sulphonated liquid wax as an emulsifying agent.

30 According to the present invention the stencil sheet comprises a fibrous base coated with a coating material consisting of a solution of esters of polysaccharides in a volatile solvent, in admixture with a liquid wax.

35 The liquid waxes consist of the liquid esters of the higher fatty acids and the higher saturated monatomic alcohols, and, therefore differ sharply from the glycerides of fatty acids.

40 The liquid waxes are further readily dis-

tinguished from the fatty oils by their low specific gravities. It is notable that their viscosity is much less influenced by variations of temperature than is the case with fatty oils.

45 The liquid waxes absorb very little oxygen from the atmosphere and therefore do not dry.

50 The typical liquid waxes are sperm oil and Arctic sperm oil (bottlenose oil).

55 In carrying out this invention, a sheet of fibrous base, such as Japanese yoshino paper, is coated or impregnated with a coating material prepared by dissolving esters of polysaccharides, such as starch acetates, mannan acetate, cellulose acetate, and cellulose nitrate, in suitable solvents and diluents, such as acetone, ethyl alcohol, butyl alcohol, benzyl alcohol, ethyl acetate, butyl acetate, amyl acetate, benzene and, toluene, or a mixture of them, a liquid wax, being added. If necessary, a tempering agent, such as fatty oils, fats, waxes, naphthenic acid glycerides, naphthenic acid and fatty acids, may be added to the coating composition. The paper base may be coated or impregnated in 60 any desired manner with the composition above described. Or, the composition may be added to the paper stuff in a mixing holander during the paper making operation.

65 70 75 The proportions of the ingredients of the coating composition may vary according to circumstances. The following is an example:

|                            | Parts by weight | 80 |
|----------------------------|-----------------|----|
| Cellulose nitrate          | 10              |    |
| Ethyl alcohol              | 5               |    |
| Butyl alcohol              | 10              |    |
| Ethyl acetate              | 15              |    |
| Butyl acetate              | 30              | 85 |
| Benzene                    | 25              |    |
| Toluene                    | 25              |    |
| Sperm oil                  | 20              |    |
| Naphthenic acid glycerides | 5               |    |
| Oleic acid                 | 5               | 90 |

The term "esters of polysaccharides" is intended to include not only one of definite esters of polysaccharides, but also a mixture of them.

In the present invention the coating material is remarkably fluid owing to the smaller viscosity of the liquid waxes. Hence, a composition of higher concentration may be obtained, with the result that a thick coating moderately soft and pliable is obtained. Moreover, the coating is permanent and is not affected by changes of temperature, permitting clear writings by the pressure of a writing machine.

As above referred to, the employment of liquid waxes in association with gelatinizing organic colloids, such as gelatine, dispersed in water has been proposed in the production of stencil sheets. In this connection, it is found that the coating composition is an emulsified mixture, and after the evaporation of water, there remains a coating consisting of a mixture of the liquid waxes and the colloids. However, the liquid waxes and the colloids do not form a homogeneous body and moreover, the compound is liable to become hard and brittle and to separate out the oily material while being stored.

According to the present invention, on the contrary, esters of polysaccharides are used, instead of gelatinous organic colloids, in association with liquid waxes, and the solution of these ingredients in volatile solvents forms a true solution. After the evaporation of the solvents there remains a pliable uniform coating which is more durable and stronger than where gelatinous organic colloids are used. The liquid wax moderately softens the coating and prevents the film from being too tough and not allowing the type to cut through.

Furthermore, it has sometimes been observed that the coating surface of stencil sheets having a coating composition of cellulose esters and fatty acid glycerides, become sticky and evolves a rancid smell, especially in the case of improperly prepared cellulose esters. This is due to the decomposition of cellulose esters started and accelerated by the rancidity of the fatty acid glycerides. In accordance with the present invention, the coating composition consists chiefly of esters of polysaccharides and a liquid wax, instead of fatty acid glycerides. Liquid wax is not liable to become rancid and, consequently, will not produce the decomposition of esters of polysaccharides and thereby the above deterioration of the coating surface of the stencil sheets.

What I claim is:—

1. A stencil sheet adapted for stencilizing by pressure comprising a base of fibrous material coated or impregnated with a composition including esters of polysaccharides and a liquid wax.

2. A stencil sheet adapted for stencilizing by pressure comprising a base of fibrous material coated or impregnated with a composition including esters of polysaccharides, a liquid wax and a tempering agent.

3. A stencil sheet adapted for stencilizing by pressure comprising a base of fibrous material coated or impregnated with a composition including esters of polysaccharides, a liquid wax and a fatty tempering agent.

In testimony whereof I affix my signature.

SHINJIRO HORII.

70

75

80

85

90

95

100

105

110

115

120

125

130